

E. BARTHELMESS,  
METHOD OF AND APPARATUS FOR PRODUCING LEAD OXID.  
APPLICATION FILED APR. 25, 1914.

1,204,537.

Patented Nov. 14, 1916.



*Witnesses,*

*G. B. Bluming*  
*W. Lyon*

*Inventor,*

*Emil Barthelmeiss*  
*by Beckers, Bynes & Sonnele*  
*his atty*

# UNITED STATES PATENT OFFICE.

EMIL BARTHELMESS, OF NEUSS ON RHINE, GERMANY.

## METHOD OF AND APPARATUS FOR PRODUCING LEAD OXID.

1,204,537.

Specification of Letters Patent. Patented Nov. 14, 1916.

Application filed April 25, 1914. Serial No. 834,426.

To all whom it may concern:

Be it known that I, EMIL BARTHELMESS, engineer, a subject of the Emperor of Germany, residing at 4 Breitestrasse, Neuss, Germany, have invented new and useful Improvements in Methods of and Apparatus for Producing Lead Oxid, of which the following is a specification.

In the previously known processes for the production of litharge, molten lead is atomized by suitable devices and is oxidized by means of a mixture of air and superheated steam, the air being sucked in by means of a steam injector and blown on to the surface of the molten lead. This has the disadvantage that the quantity of steam which it is necessary to introduce for the complete oxidation, cannot be determined, so that in most cases it is necessary to work with an excess of steam, in consequence of which the lead oxid exhibits a more or less high percentage of moisture. Moreover the apparatus which work according to this method and which have a large oxidation chamber are arranged in an impracticable manner inasmuch as it is very difficult to heat them uniformly. In consequence of this, incomplete oxidation and the formation of incrustations on the inner surfaces of the oxidation chamber frequently result; in the latter case the removal of such incrustations can only be effected with difficulty. Furthermore the separation of the properly oxidized and badly oxidized lead can only be effected by the aid of particularly high oxidation chambers, which exhibit the last named defects in an especially high degree. All these disadvantages are avoided by the present invention wherein cold water or water which has been previously heated is used instead of steam. This water is introduced into the stream of gas necessary for oxidation drop by drop and in measurable quantities. In consequence of this the proportions of lead to be oxidized and water to be added, which are most favorable for the oxidation, can be determined, while, on the other hand the whole plant is considerably simplified by the omission of a steam generator or superheater respectively.

The oxidation chamber is easily accessible and is heated uniformly on all sides by means of a fan-like stirring device, which is formed to closely fit the interior surface of the said oxidation chamber, whereby any deposition of oxid on the heating surfaces

is prevented and the best conditions for oxidation are insured. The oxidizing stream of gas, which is sucked in by the mixing device at the front end of the oxidation chamber and which may consist of air, oxygen or any desired mixture of oxygen, serves at the same time for the expulsion of the lead oxid dust which has been formed at the opposite end. Before its entry into the oxidation chamber the said stream of gas may, for the purpose of preliminary heating, be led through suitable heating channels arranged in the brickwork of the heating apparatus and after leaving the oxidation chamber and depositing the lead oxid dust the said stream of gas may be brought back to the inlet through suitable pipes protected against heat losses. The incompletely oxidized lead, which is deposited in the rear part of the oxidation chamber is returned to the bath of molten lead by means of the said mixing device. This mixing device serves thus on the one hand for atomizing the lead and for scraping off and conveying back the badly oxidized lead, while, on the other hand, it causes the passage of a stream of gas through the apparatus, which stream contains the quantity of oxygen necessary for the oxidation and at the same time effects the separation of the lead oxid contaminated with metal from the litharge and the expulsion of the latter.

The annexed drawing shows in vertical section one constructional form of a device suitable for carrying out the present process.

*a* is a pear-shaped containing vessel of iron or fireproof material, which is arranged in an inclined position and is tapered off toward one end. This containing vessel serves as an oxidation chamber and is in direct connection with a melting pot *b*, into which the lead to be melted is introduced in the form of bars through lateral openings *c*. The pot *b*, which is heated by means of a suitable heating device *d*, is completely surrounded, as is also the containing vessel *a*, by brickwork in such a manner that the hot gases can spread over all the surfaces of the apparatus without hindrance and heat the same uniformly.

A spindle *e* is mounted in the axis of the vessel *a*. This spindle runs in bearings formed at the ends of the vessel *a* and is caused to rotate through the agency of a pulley *f* which is driven from any suitable

source of power. The spindle *e* is provided with a stirring device which serves for atomizing the lead melted in the pot *b*. The said stirring device is formed so as to closely fit the inner surface of the oxidation chamber. The stirring device consists of a centrifugal wheel *g* arranged at the front end of the spindle *e* in such a manner as to dip into the molten lead in the pot *b*, the rear part of the scraper comprising a series of conically disposed blades *h*. These blades and also the vanes of the centrifugal wheel, are adapted to prevent the formation of a deposit of lead oxid on the heating surfaces and to transport the badly oxidized or unoxidized lead back to the bath of molten lead.

The centrifugal wheel *g* is made in the form of a fan which sucks the stream of gas necessary for the oxidation of the lead through the central inlet *i*. In order to heat the stream of gas sufficiently before its admission it is led through the inlet at *l* into the heating channels *k* formed in the brick-work and thence through the pipe *m*, through which latter the water necessary for the oxidation of the lead is introduced by means of a measuring vessel *n* provided with a dropping device. This arrangement renders it possible to regulate exactly the proportion between the amount of lead to be oxidized and the necessary quantity of water to be added.

The gas streaming through the oxidation chamber with increasing velocity carries the lead oxid which has been formed toward the outlet *o* at the opposite end, this outlet being connected to a transporting device *p*, by means of which the lead oxid is conveyed away to suitable collecting funnels (not shown on the drawing). The dust which is also carried out with the litharge is deposited in the depositing chamber *q*, which is connected at *r* to a dust extracting plant. If pure oxygen be employed as the oxidizing gas, then the depositing chamber *q* may be connected by means of a pipe *S* (shown in dotted lines) which is also protected against heat losses, to the pipe *m*, in order to return the unused oxygen to the inlet *i* and thus employ it again. This arrangement renders it possible at the same time to regulate the velocity of the gas necessary to expel the lead oxid.

55 Claims:

1. The method of producing lead oxid consisting in atomizing molten lead in a uniformly heated chamber, passing a stream of gas containing oxygen through said chamber, adding water drop by drop in measured quantities to said gas, and drawing off the gas with lead oxid dust in suspension; substantially as described.

2. The method of producing lead oxid consisting in atomizing molten lead in a uni-

formly heated chamber, passing a stream of gas containing oxygen through said chamber, adding water drop by drop in measured quantities to said gas, drawing off the gas with lead oxid dust in suspension, and separating the lead oxid dust from the gas, substantially as described. 70

3. The method of producing lead oxid consisting in atomizing molten lead in a uniformly heated chamber, passing a stream of gas containing oxygen through said chamber, adding water drop by drop in measured quantities to said gas, drawing off the gas with the lead oxid dust in suspension, separating the lead oxid dust from the gas and 75 repassing the gas through the chamber, substantially as described.

4. The method of producing lead oxid consisting in admitting heating gases to direct contact with all the outer surfaces of an oxidation chamber, passing a heated stream of gas containing oxygen through said chamber, adding water drop by drop in measured quantities to said stream, drawing off the gas with the lead oxid dust in suspension, separating the dust from the gas, and regulating the velocity of the gas for expelling the oxid, substantially as described. 90

5. The method of producing lead oxid 95 consisting in atomizing molten lead in a uniformly heated chamber, passing a stream of gas containing oxygen through said chamber, adding water drop by drop in measured quantities to said gas, drawing 100 off the gas with lead oxid dust in suspension, and returning the unoxidized lead from the chamber back to the path; substantially as described.

6. Apparatus for producing lead oxid, 105 comprising an oxidizing chamber, a molten lead bath in said chamber, and a mixing device having a fan connected thereto and arranged in said chamber, said mixing device closely fitting the walls of the chamber, dipping into the bath of metal, and serving to suck in a stream of gas containing oxygen and scrape off and convey back to the molten bath the incompletely oxidized lead deposited on the walls of the chamber, 110 substantially as described. 115

7. Apparatus for producing lead oxid, comprising a pear-shaped oxidizing chamber arranged in an inclined position and tapered off toward one end, a lead melting pot 120 in direct communication with said chamber, the said chamber and the said melting pot being inclosed in a common heating chamber, and means in said chamber for atomizing the lead in said chamber and for sucking in gas containing oxygen, substantially as described. 125

8. Apparatus for producing lead oxid, comprising an inclined chamber having an oxidizing gas supply inlet at one end and an 130

outlet at the opposite end, a molten lead bath in said chamber, a driving spindle extending centrally through said chamber, and a centrifugal wheel on said spindle which 5 dips into the bath of molten lead said centrifugal wheel being made in the form of a fan, and being arranged directly adjacent to the gas inlet, substantially as described.

9. Apparatus for producing lead oxid, 10 comprising an inclined chamber having an oxidizing gas supply inlet at one end and an outlet at the opposite end, a molten lead bath at the inlet end, a driving spindle extending centrally through said chamber, a 15 centrifugal wheel on said spindle arranged opposite the gas inlet and adapted to dip into said molten bath, and projecting blades on said wheel arranged to closely fit the internal surface of the chamber, substantially 20 as described.

10. Apparatus for producing lead oxid, comprising an inclined chamber, a molten bath in said chamber, a rotary fan-like mixing device arranged in said chamber, said 25 fan-like device closely fitting the walls of the chamber, and a gas supply to said chamber, said inclined chamber being surrounded by a heating chamber made of brickward and said gas supply being led through channels 30 formed in said brickwork, substantially as described.

11. Apparatus for producing lead oxid, comprising an inclined conical chamber surrounded by a heating chamber made of 35 brickwork, a molten bath in said chamber, a rotary fan-like mixing device arranged in said chamber opposite a gas supply opening and adapted to dip into said bath, gas supply channels in the walls of brickwork 40 leading to said supply opening, a gas and lead oxid dust outlet, means for separating the gas from the lead oxid dust, and means for returning the gas to the supply opening, substantially as described.

45 12. Apparatus for producing lead oxid comprising an inclined conical chamber, a molten lead bath in said chamber, means for atomizing the lead in said bath for causing a stream to be drawn in said chamber, and

for scraping off deposits of lead oxid on the 50 walls of the chamber, means for separating the lead oxid dust from the stream of gas which has passed through the chamber, heat insulated funnels, and transporting devices for carrying the lead oxid to said funnels, 55 substantially as described.

13. Apparatus for producing lead oxid, comprising an oxidizing chamber, having a gas outlet at one end and a gas inlet at the other end, a lead bath at said inlet end, 60 a fan-like mixing device above said bath and adjacent to said gas inlet, a water supply pipe on the suction side of said fan, and measuring devices in connection with said water supply pipe, substantially as de- 65 scribed.

14. Apparatus for producing lead oxid comprising an oxidizing chamber, a molten lead bath in said chamber, a gas inlet leading thereto, means for atomizing the lead in 70 said bath, means for sucking in a current of gas containing oxygen and admixed with water, said gas carrying off the lead oxid dust, and means for regulating the velocity of the gas passing through the chamber. 75

15. Apparatus for producing lead oxid, comprising an oxidizing chamber having a gas inlet, a molten lead bath in said chamber, a suction fan arranged in front of said gas inlet, a water supply pipe, and means 80 for regulating the amount of water passing through said pipe, substantially as described.

16. Apparatus for producing lead oxid comprising a chamber, means for uniformly 85 heating said chamber, a pot for melting lead in said chamber, means for passing a stream of gas through said chamber, means for adding water in measured quantities to said gas, and means for drawing off the gas with a 90 lead oxid dust; substantially as described.

In testimony whereof I have signed my name to this specification in the presence of two subscribing witnesses.

EMIL BARTHELMESS.

Witnesses:

HELEN NUFER,  
ALBERT NUFER.